

# United States Patent [19]

Restall et al.

[11] 3,922,168

[45] Nov. 25, 1975

[54] **INTERMETALLIC COMPOUND MATERIALS**

[75] Inventors: **James Edward Restall**, Frimley; **Michael James Douglas Weaver**, Fleet, both of England

[73] Assignee: **National Research Development Corporation**, London, England

[22] Filed: **Jan. 10, 1974**

[21] Appl. No.: **432,392**

**Related U.S. Application Data**

[63] Continuation-in-part of Ser. No. 256,026, May 23, 1972.

[30] **Foreign Application Priority Data**

May 26, 1971 United Kingdom..... 17150/71  
Jan. 12, 1973 United Kingdom..... 1676/73

[52] **U.S. Cl.** ..... **75/171; 75/170; 148/32;**  
148/32.5

[51] **Int. Cl.<sup>2</sup>** ..... **C22C 19/05**

[58] **Field of Search** ..... **75/171, 170; 148/32, 32.5**

[56] **References Cited**

UNITED STATES PATENTS

3,617,397 11/1971 Maxwell..... 75/170  
3,767,479 10/1973 Tarshis..... 75/171

FOREIGN PATENTS OR APPLICATIONS

1,011,785 12/1965 United Kingdom  
1,019,679 2/1966 United Kingdom  
1,036,148 7/1966 United Kingdom  
1,065,770 4/1967 United Kingdom

1,087,051 10/1967 United Kingdom

*Primary Examiner*—R. Dean  
*Attorney, Agent, or Firm*—Cushman, Darby & Cushman

[57] **ABSTRACT**

An intermetallic compound material based on tri-nickel aluminide which may be produced by standard vacuum melting techniques, is composed of a first group of constituents in which the nickel is partly replaced by at least one of the elements chromium, cobalt, molybdenum and tungsten and a second group of constituents in which the aluminium is partly replaced by hafnium and by at least one of the elements titanium, niobium and tantalum, the material containing the constituents in the proportions, by atomic percentage,

first group of constituents 72 to 83

second group of constituents 17 to 28

One preferred composition of the intermetallic compound material contains elements of the said first and second groups in the following ranges specified below, in atomic per cent,

|            |          |           |          |
|------------|----------|-----------|----------|
| Nickel     | 60 to 80 | Aluminium | 12 to 26 |
| Chromium   | 2 to 6   | Titanium  | 0 to 12  |
| Cobalt     | 0 to 12  | Niobium   | 0 to 6   |
| Molybdenum | 0 to 3   | Tantalum  | 0 to 6   |
| Tungsten   | 0 to 3   | Hafnium   | Up to 6  |

The intermetallic compound material may contain carbon, boron, and zirconium as trace elements.

**4 Claims, No Drawings**

## INTERMETALLIC COMPOUND MATERIALS

This application is a continuation-in-part of our pending application Ser. No. 256,026 filed May 23, 1972 for "Intermetallic Compound Materials".

This invention relates to intermetallic compound materials based on tri-nickel aluminide ( $Ni_3 Al$ ) and which include hafnium.

The majority of high temperature structural components currently used in gas turbine aero engines are made from nickel-base alloys strengthened primarily by the precipitation of  $Ni_3 Al$  (gamma-prime) throughout the nickel (gamma) matrix. During recent years, the strengths of such alloys have been improved by increasing the stability and volume fraction of the gamma-prime precipitate through the introduction of relatively large quantities of elements such as tungsten, molybdenum, tantalum, niobium and titanium. This has involved reduction of the nickel and chromium content, the strength improvements thus being obtained at the expense of corrosion resistance. It is known that in addition to its precipitation strengthening role, the gamma-prime phase present in commercial precipitation-hardened nickel-base alloys has good corrosion resistance at high temperatures.

Binary  $Ni_3 Al$  has little worthwhile high temperature strength and is fairly brittle but alloys based on  $Ni_3 Al$  containing additional alloying elements can combine the high corrosion resistance of  $Ni_3 Al$  with the strength and ductilities of modern precipitation-hardened nickel-base alloys at higher temperatures than the latter can withstand.

An intermetallic compound material based on tri-nickel aluminide according to the invention is composed of a first group of constituents in which the nickel is partly replaced by at least one of the elements chromium, cobalt, molybdenum, and tungsten and a second group of constituents in which the aluminum is partly replaced by hafnium and by at least one of the elements titanium, niobium and tantalum, the material containing the constituents in the proportions by atomic percentage,

First group of constituents 72 to 83  
Second group of constituents 17 to 28

Preferably the constituents are in the following ranges (specified in atomic per cent):-

|            |          |           |          |
|------------|----------|-----------|----------|
| Nickel     | 60 to 80 | Aluminium | 12 to 26 |
| Chromium   | 2 to 6   | Titanium  | 0 to 12  |
| Cobalt     | 0 to 12  | Niobium   | 0 to 6   |
| Molybdenum | 0 to 3   | Tantalum  | 0 to 6   |
| Tungsten   | 0 to 3   | Hafnium   | Up to 6  |

Additional trace elements are 0.05 to 0.5 carbon, 0.01 to 0.1 boron, and 0.01 to 0.2 zirconium (all atomic percentages).

Intermetallic compound materials according to the invention can be produced by standard vacuum melting techniques. As a typical example, nickel, cobalt, carbon and boron are melted under vacuum and when the melt is fully degassed, chromium and any refractory metals are added under a partial pressure of argon. Aluminium, hafnium, titanium and zirconium are then added under vacuum and the metal cast into ingot form. Conventional casting techniques have produced

materials having acceptable high temperature strengths and ductilities. Uni-directional solidification in which a temperature gradient is induced by progressive cooling in order to control crystalline growth to give a columnar structure has been found to give increased strength and ductility.

The following is the composition expressed in atomic per cent an example of an intermetallic compound material according to the invention:

|    |          |         |           |      |           |      |
|----|----------|---------|-----------|------|-----------|------|
| 10 | Nickel   | Balance | Aluminium | 16.5 | Carbon    | 0.5  |
|    | Chromium | 3.5     | Hafnium   | 0.5  | Boron     | 0.05 |
|    | Cobalt   | 7.1     | Tantalum  | 3.6  | Zirconium | 0.05 |
|    | Tungsten | 0.9     |           |      |           |      |

15 This composition is representative of those believed to give good combinations of desirable properties, but is not intended to be exclusive. The composition when conventionally cast using standard vacuum casting procedures, has the following properties:-

TABLE I

| 25 | Test temperature °C | Tensile Properties |    | % Elongation |
|----|---------------------|--------------------|----|--------------|
|    |                     | UTS (tsi)          | 57 |              |
|    | 20                  | 700                | 58 | 10<br>3      |

TABLE II

| 30 | Test conditions | Creep Properties |    | % Elongation |
|----|-----------------|------------------|----|--------------|
|    |                 | Life (hours)     | 76 |              |
|    | 4 tsi - 1100°C  | 76               | 6  |              |
|    | 8 tsi - 1000°C  | 145              | 10 |              |
|    | 20 tsi - 900°C  | 171              | 6  |              |

TABLE III

| 40 | Total weight gain after 425 hours (mg/cm <sup>2</sup> ) | Oxidation Properties |     | Test temperature °C |
|----|---------------------------------------------------------|----------------------|-----|---------------------|
|    |                                                         | 1.0                  | 3.6 |                     |
|    |                                                         | 1.0                  | 3.6 | 1100                |
|    |                                                         |                      |     | 1200                |

45 Tri-nickel aluminide exists only over a very narrow range in the Ni-Al phase diagram, and it is difficult to cast a component with a single phase structure. All the compositions according to the invention therefore are 50 likely to contain, both in the conventionally cast condition and after unidirectional solidification, small quantities of nickel (gamma) and Ni-Al (beta) type phase, either separately or together. Metal carbides and borides are also likely to be present.

55 I claim:

1. In an intermetallic compound material based on tri-nickel aluminide consisting essentially of constituents in proportion by atomic percent:

first constituents 72-83% wherein the elements are present in the range, in atomic percent,

|            |       |
|------------|-------|
| Nickel     | 60-80 |
| Chromium   | 2-6   |
| cobalt     | 0-12  |
| Molybdenum | 0-3   |
| Tungsten   | 0-3   |

60 second constituents 17-28% wherein the elements are present in the range, in atomic percent

|          |       |
|----------|-------|
| Aluminum | 12-26 |
| Titanium | 0-12  |
| Niobium  | 0-6   |
| Tantalum | 0-6   |

5

said aluminum partly replaced by at least one of the elements selected from the group consisting of titanium, niobium and tantalum, the improvement which comprises including from 0.5 to 6 atomic percent hafnium in said second constituents.

2. An intermetallic compound material based on tri-nickel aluminide consisting essentially of, atomic percentage:

|             |       |      |
|-------------|-------|------|
| A. chromium | about | 3.5  |
| cobalt      | about | 7.1  |
| tungsten    | about | 0.9  |
| B. aluminum | about | 16.5 |
| hafnium     | about | 0.5  |
| tantalum    | about | 3.6  |
| and         |       |      |
| carbon      | about | 0.5  |

20

-continued

|           |          |      |
|-----------|----------|------|
| boron     | about    | 0.05 |
| zirconium | about    | 0.05 |
| nickel    | balance. |      |

3. An intermetallic compound material as claimed in claim 2 including carbon, boron and zirconium as trace elements in proportions by atomic percentage,

|    |           |              |
|----|-----------|--------------|
| 10 | Carbon    | 0.05 to 0.5  |
|    | Boron     | 0.01 to 0.1  |
|    | Zirconium | 0.01 to 0.2. |

4. An intermetallic compound material as claimed in claim 1 including carbon, boron and zirconium as trace elements in proportions, by atomic percentage,

|    |           |              |
|----|-----------|--------------|
| 15 | Carbon    | 0.05 to 0.5  |
|    | Boron     | 0.01 to 0.1  |
|    | Zirconium | 0.01 to 0.2. |

\* \* \* \* \*

25

30

35

40

45

50

55

60

65